

June 9, 1931.

J. E. BOND

1,808,830

METHOD OF AND APPARATUS FOR DIGESTING WOOD

Filed May 27, 1929



## UNITED STATES PATENT OFFICE

JOSEPH E. BOND, OF APPLETON, WISCONSIN

## METHOD OF AND APPARATUS FOR DIGESTING WOOD

Application filed May 27, 1929. Serial No. 366,295.

My invention relates to the art of pulp production and particularly to an improvement in the construction and operation of digesters.

5 In the sulphite treatment of wood chips, the Ritter-Kellner or direct process and apparatus are commonly employed. This process admittedly has many shortcomings in the 10 quantity of cellulose produced and in the efficiency of the process as a whole but is used in preference to other more efficient methods because of the relatively quicker time within which pulp may be produced.

The process of digestion consists in subjecting 15 the chips to the action of an acid, and depends for its success on the difference in solubility of the important constituents of wood: that is, the lignin, sugar and resin of wood are relatively more soluble in the particular 20 acid employed than cellulose. However, cellulose under extreme conditions of strength of acid, temperature, pressure and time is soluble in the same acid and, therefore, the process must be carried on in such manner 25 that the more soluble constituents may be attacked and dissolved without impairing the strength and hydration capacity of the cellulose.

Inasmuch as the wood must for practical 30 purposes be treated in the form of chips or other divisions of substantially uniform size the difficulty encountered is that of securing penetration of the acid to the interior parts of the small body of wood before the exterior 35 portions have been treated to such an extent that the quality of the cellulose fibers is harmed. Experience has shown that during the first hour or two in the digester, the temperature should be 110° C. in order to prevent 40 the formation of an insoluble lignin compound around the chips which renders the chips impervious to subsequent treatment. However, it is desirable to raise the temperature of the mass within the digester as quickly 45 as possible. This involves the admittance of steam at high pressure and usually there is a percentage of burned or useless chips that have been rendered useless by proximity to the steam inlet.

50 It is a well known physical fact also that

solubility is greatly increased where there is efficient agitation; this for the reason that if the solvent and the body to be dissolved remain quiescent the solvent immediately around the body becomes saturated and its 55 efficiency is lost. In the processes heretofore employed, circulation of the chips has been effected solely by means of steam jets, although in some cases the acid without the chips has been circulated, as in the Mitscherlich process.

My invention contemplates, in effect, a combination of the advantages of both the Ritter-Kellner and the Mitscherlich processes, and, in addition, a radical departure 65 from the practice commonly employed. For example, I accomplish the quick saturation and cooking of the direct process with the advantages of the indirect process.

The invention will be more readily understood by reference to the accompanying drawings, and will be more specifically pointed out in the subsequent description of the apparatus employed.

In the accompanying drawings, 75 Fig. 1 is a vertical sectional view through a digester constructed in accordance with my invention, the illustration being somewhat diagrammatic as to certain details; and

Fig. 2 is a sectional view on the line 2—2 80 of Fig. 1.

The apparatus which I prefer to employ consists of a lined shell 10 having a covered inlet opening 11 at the top through which the chips are admitted. The casing has a 85 conical bottom 12 and is supported in the usual manner.

As a means for carrying out the process of my invention, I make a departure from the usual digester construction by providing a large centrally disposed pipe 13 having an open top that terminates short of the upper end of the digester. The lower end is in communication with the discharge outlet of a centrifugal or screw pump 14, the impeller of which is indicated at 15. The impeller is mounted on a relatively long shaft 16 having outboard bearings 17—18 and actuated by a motor 19. The inlet portion 20 of the pump casing is extended to receive a 100

plurality of ship propellers 21 mounted on the shaft 16, having the function of disintegrating the chips, breaking up any lumps or clumps of material and generally assisting 5 in the agitation. The inlet pipe 22 is in communication with the lower end of the conical portion of the shell.

Arranged exteriorly of the digester in a suitable casing 23 is an acid heating tank 10 containing steam coils 24. A pipe 25 connects with the inlet pipe 22 and a centrifugal pump 26 in the pipe line 25 withdraws acid from the digester, passes it through the tank and returns it through the pipe 27 to the inlet casing 22 adjacent to the zone of operation 15 of the propellers 21. Fresh acid may be admitted through the pipe 25a, as may be necessary at the start of operations.

Also connected to the casing 21 is a pipe 20 28 adapted to admit steam if and when required.

Notwithstanding that the digester is filled with chips at the start of operation, the bulk 25 will be reduced as the operation proceeds. I have therefore extended the pipe 13 near to the top of the casing to insure the flow of acid over the top of the chips. However, as 30 digestion proceeds, the bulk will be lessened and there is no necessity for raising the material materially above the level in the digester. I have, therefore, provided means such as the sleeve 29 within the pipe for opening and closing ports 30 when it is unnecessary to raise the material to the top of the pipe. 35 The sleeve may be operated by means of a screw 31 having an exterior handwheel and connected to a shaft 32 rigid with the sleeve.

The operation of the apparatus in carrying out my improved process is as follows:

40 The digester and the pipe 13 are filled with chips in the usual manner. After the filling opening is closed, acid is pumped through the pipe 25a and 27 and caused to rise in the tube 13. The chips in the tube being loosely packed will permit the acid to rise around them and it will overflow and spread itself over the top surface of the chips in the space around the tube. The pump 14 being in 45 operation, as soon as acid reaches the bottom 50 it will, together with some of the chips, be again directed into the central pipe and the circulation of both the chips and the acid will begin. If the chips are dry, steam will be admitted through the pipe 28 along with the acid. The rapid movement of the chips and acid and the complete agitation at the 55 point of admission of the steam will prevent burning, as the steam will be condensed very 60 quickly.

In order to quickly raise the temperature of the mass within the digester without diluting the acid with an excessive amount of steam, I withdraw acid through the pipe 25 65 and pass it through the heater returning it

to the pump inlet in properly heated condition.

By indirectly heating the acid and by thorough agitation of the digester contents, the time of cooking is materially reduced and the yield of cellulose is greatly increased. The cost of operation is also materially reduced for the reason that the cooking acid is not extensively diluted by water from condensed steam. Thus there is a lessening of 75 expense in the recovery of SO<sub>2</sub>. By effective circulation and the accurate control of temperature during the penetration or saturation period, I am able to reduce the percentage of burned chips, slivers, and tailings and the mechanical device employed for circulation assists materially in the disintegration of the wood chips.

The apparatus employed is typical only and other forms may be devised and utilized 85 to advantage without departure from the spirit of my invention.

I claim:

1. The method of operating a digester having a vertical open top tube therein which 90 consists in charging chips into the digester and tube then delivering hot acid to the bottom of the tube and causing it to rise and overflow over the top of the chips in the space around the tube, then continuously 95 pumping acid and chips from the bottom of the space around the tube and discharging said acid and chips upwardly through said tube, withdrawing cooled acid from the digester, indirectly heating the same at a point 100 exterior of the digester and returning the heated acid to the moving body of material.

2. The method of operating a digester having a vertical open top tube therein which 105 consists in charging chips into the digester and tube then delivering hot acid to the bottom of the tube and causing it to rise and overflow over the top of the chips in the space around the tube, then continuously 110 pumping acid and chips from the bottom of the space around the tube and discharging said acid and chips upwardly through said tube, withdrawing cooled acid from the bottom of the digester and supplying hot acid to 115 the body of material that is being discharged into said tube.

3. The method of operating a digester which consists in supplying chips thereto, then supplying hot acid and steam while continuously and mechanically circulating the 120 contents of the digester until the temperature of the contents is raised to approximately 105° C., then continuing the circulation of the contents and maintaining the temperature substantially constant until saturation is complete, then raising the temperature to a proper coking temperature and continuing the circulation of the chips and acid.

4. The combination of a digester having 125

a vertical open top tube therein, a pump having its inlet connected to the bottom of the space surrounding the tube and its outlet connected to said tube, means for supplying hot acid to the digester at a point adjacent to the inlet to said pump, and means in the intake for disintegrating the chips.

5. The combination of a digester having a vertical open top tube therein, a pump having its inlet connected to the bottom of the space surrounding the tube and its outlet connected to said tube, means for supplying hot acid to the digester at a point adjacent to the inlet to said pump, and a ship propeller 10 in the intake for disintegrating said chips 15 before they enter the pump.

6. The combination of a digester having a vertical open top tube therein, a pump having its inlet connected to the bottom of the space 20 surrounding the tube and its outlet connected to said tube, and means for withdrawing cooled acid from the bottom of the digester, heating the acid exteriorly of the digester and returning the heated acid to the 25 pump.

7. The combination of a digester having a vertical open top tube therein, a pump having its inlet connected to the bottom of the space surrounding the tube and its outlet connected 30 to said tube, means for continuously withdrawing cooled acid from the lower portion of the digester, means for indirectly heating the withdrawn acid, and means for returning the heated acid to the moving body 35 of chips and acid passing through the pump.

8. In a digester the combination with the casing of a vertical open top pipe therein, a pump having its outlet connected to the pipe and its inlet connected to the bottom of the 40 casing, and means for varying the effective length of the pipe.

9. In a digester the combination with the casing of a vertical open top pipe therein, a pump having its outlet connected to the pipe 45 and its inlet connected to the bottom of the casing, means providing a port in the pipe at a point below its upper end, and means operable from the exterior of the digester for opening said port when the level of material 50 in the digester is adjacent to said port.

In testimony whereof I have affixed my signature.

JOSEPH E. BOND.